

## UNITED STATES PATENT OFFICE

2,020,936

PROCESS OF PRODUCING A MINERAL OIL  
SUBSTITUTE PAINT VEHICLE

Giovanni Fiore, New York, N. Y.

No Drawing. Application July 10, 1934,  
Serial No. 734,511

2 Claims. (Cl. 134—56)

My invention relates to the manufacture, from crude mineral oil or any of its fractions, distillates or residuals of an oxidizable mineral oil which may be practically and economically applied to various uses in the mechanical arts, especially also as an oxidizable drying vehicle for paint pigments or as a plain varnish or constituent of plastic materials or printing inks. One of the greatest advantages of this product is that it may be used as an adequate inexpensive substitute for linseed oil and other similar oils, capable of oxidizing and drying, while its selling price may be less than a fourth of that of linseed oil. Up to comparatively recent times mineral oils could not be used like certain vegetable oils or organic fats as vehicles for pigments or bases for lacquers, having no drying qualities, and even the addition of driers or oxidizing agents to them did not remedy this deficiency. The numerous attempts to convert various forms or derivatives of such mineral oils into oxidizable drying oils have been only partly successful, and the difficulties become obvious if we investigate the phenomena taking place when a paint or a lacquer with a suitable drying base solidifies. Assuming, for example, a pigment carrier like boiled linseed oil or castor oil (the latter being used in coating compositions for artificial leather), the drying process is not accomplished by the loss and evaporation of water, but by the oxidation of liquid fatty acids (oleic, linolic, linolenic, isolinolenic) or solid acids (palmitic and stearic) in linseed oil or other vegetable oils. These acids, being exposed to the air, tend to absorb oxygen, and form solid oxides. Certain glycerides present in the mineral oils promote this solidifying process by esterifying the free aldehyde-fatty acids present and act therefore as excitors of oxidation. The glycerides of linolic, linolenic, isolinolenic or oleic acids enter completely into this oxidizing process while the glycerides of other acids act in a similar way. The final products of the oxidation of linseed oil, commonly called "Linoxyn", are probably a mixture of solid oxides of linolenic and isolinolenic acids, oxidized glycerides and a trace of glycerine.

In mineral oils, however, these fatty acids are absent, and therefore they exhibit no drying or oxidizing power.

As far as these mineral oils and their related asphaltic compounds are concerned, one usually distinguishes two main classes, one class which comprises saturated hydrocarbons, having a paraffin basis (petroleum oils, found east of the Mississippi River, Pennsylvania, etc., are of this

class) and one class, having an asphaltic base and consisting largely of unsaturated hydrocarbons or olefins (Texas, Gulf or California oils). While both kinds have in themselves no drying qualities, experiments to oxidize mineral oils of the second class or at least their derivatives have been partly successful, while the lighter and more liquid oils of the first class—which contained more or less paraffins—have proven more recalcitrant to any oxidizing treatment. Furthermore, rather high temperatures seemed necessary but at elevated temperatures considerable darkening and even decomposition takes place. The broader object of the present invention is to devise a method whereby mineral oils with a paraffin basis can be just as successfully converted into oxidizable oils at a comparatively low temperature (100° C.) and within a short time, as mineral oils, in which the paraffins are missing, or from which they have been artificially removed, and both kinds in the same way and same period of time.

The leading principle of my invention is that I introduce the missing elements, the fatty acids, indirectly by means of a suitable vehicle into the mineral oil. This is the first step, but in itself would not be sufficient even if a catalyst were added, to induce complete oxidation. The second concurrent principle of my method is that instead of simple oxygen I use the more potent form "ozone" ( $O_3$ ) and submit the mineral oil containing the fatty acids to a current of ozone.

But what in my estimation is the most potent agent to complete the oxidizing process, once the favorable preliminary conditions are given, as above described, is the addition of alcohol and nitric acid in combination. Alcohol itself has a strong power of developing oxygen, but its combination with nitric acid or derivatives of the latter increases, as I found, this power in a surprising manner.

Considering the objects of my invention more in detail, it may be said that—

The first object of my invention is to devise a method whereby mineral oil of any origin, whether having an asphaltic base or a paraffin base, may be brought into an oxidizable form.

Another object of my invention is to devise a method whereby fractional distillates or residuals of a normally unoxidizable mineral oil may be converted into an oxidizable oil.

A further object is to convert a normally unoxidizable residue of crude oil, from which the paraffins have been removed by fractional distillation, into an oxidized or oxidizable form.

A further object is to devise a method whereby the residue of a natural mineral oil wherefrom certain valuable constituents have been removed by the so-called "cracking" process, may be converted into a valuable product in the form of an oxidizable mineral oil.

Another object is to devise a method whereby mineral oil of any constituency, whether in the natural state, or after undergoing fractional distillation, may be converted into an oxidizable oil without the necessity of previously removing therefrom any constituents, generally considered recalcitrant to an oxidizing process, like paraffins, etc.

15 A further object of my invention is to manufacture from crude oil of any description, a vehicle which can be used for pigments of any shade or chemical composition and which will impart to such pigments a drying quality.

20 A further object of my invention is to manufacture from crude oil or the residues of such crude oil from fractional distillation, a vehicle for paint pigments, printers' ink, lacquers, etc. in the shape of an oxidizable mineral oil.

25 Another object of my invention is to manufacture from crude oil or the residues from fractional distillation of crude oil a serviceable and non-expensive substitute for linseed oil.

30 A further object of my invention is to manufacture from crude oil or its fractional derivatives an oxidizable oil which can be used advantageously as a substitute for any vegetable oils commonly used as vehicles for pigments.

35 Another more specific object of my invention is to provide an admixture, which, when blended with crude oil or any of its fractional derivatives, and combined with them in a certain definite way, will impart to said oil or its derivatives the quality of spontaneous oxidation.

40 Another object is to provide such admixture in the form of a vegetable oil which will contain the active ingredients, i. e., the fatty acids, in a certain suitable definite proportion.

45 A further object of my invention is to initiate the oxidation of said fatty acids by the introduction of oxygen in a specially potent form.

A similar object is to initiate the oxidation of said mixture of crude oils and fatty acids by the introduction of oxygen in the form of ozone.

50 A similar object is to initiate the oxidation of said fatty acids by "ozonizing" the air brought into intimate contact with them during their first stage of oxidation.

55 A further object of my invention is to provide certain admixtures for the crude oil or its derivatives, while undergoing the initial steps of oxidation, which will serve as powerful stimulants in this oxidation process.

60 Other more specific objects and advantages of my invention will appear as the nature of my method is better understood and the steps are explained in detail.

65 The disclosure made the basis of exemplifying the present inventive concept suggests a practical embodiment thereof, but the invention is not to be restricted to the exact details of this disclosure nor to the exact quantities set forth in the formulas which are to be taken rather as illustrative than as restrictive.

70 It is also to be understood that the various steps of the process disclosed may be separately applicable despite their cooperation herein shown, and that also all possible chemical equivalents instead of the media enumerated would

come within the legitimate scope of the invention.

I shall now describe my process in detail. For the sake of a better understanding and distinction of principal steps, my process may be divided into three parts, listed under A, B and C. 5

"A" comprises the preparation of the admixture; that is, of the vegetable oil, as the carrier of the fatty acids in proper proportion, to be mixed afterwards into the crude oil or fractional residue of the crude oil, the addition of certain metal oxide driers to the crude oil, besides a "protective colloid" to prevent precipitation, and the intimate combination of these ingredients by heating at low temperature. 15

"B" comprises the heating of the crude oil or whatever fractional part or residue of it is to be treated, the incorporation of the admixture prepared according to "A" into it, and the treatment of this compound mixture by ozone. 20

"C" comprises the treatment of the ozonized compound by a mixture of alcohol and nitric acid, the addition of a volatile drier and the ageing of the finished product. 25

#### A.—Preparation of the admixture

Although there is apparently a great choice of oxidizable vegetable oils which contain fatty acids in more or less suitable proportions and which therefore could be used advantageously to 30 carry out my process, there are to be found among the available oils such which also contain "methylenic ether", and this ingredient I found to be especially helpful in oxidation. This ingredient is, for example, to be found in Sesamum 35 Indicum oil which contains its fatty acids also in other respects in a proportion that might be taken as a model. Such oil, if of best quality, will approximately contain:

|                                       | Per cent |
|---------------------------------------|----------|
| Oleic acid, $C_{17}H_{33}COOH$        | 17.50    |
| Palmitic acid, $C_{16}H_{32}O_2$      | 8        |
| Stearic acid, $CH_3(CH_2)_{16}CO_2H$  | 8        |
| Linolic acid, $C_{18}H_{32}O_2$       | 30       |
| Iso-linolenic acid, $C_{18}H_{30}O_2$ | 27       |
| Methylenic ether, $(CH_3)_2O$         | 45       |
| Glycerine, $C_3H_5(OH)_3$             | 5        |
|                                       | 4.5      |

Of this vegetable oil I take a quantity which would be equal to about 10% of the predetermined total quantity of the finished product. I 50 heat this oil to a temperature of about 65° C. while I add to it certain driers in the form of metallic oxide. For example—

|                                                                                            | Per cent |
|--------------------------------------------------------------------------------------------|----------|
| Lead resinate (fused or precipitated and dissolved in a volatile solvent or vegetable oil) | 55       |
| Cobalt resinate                                                                            | 1        |
| Manganese resinate                                                                         | 1        |

I reserve, however, the right to use other metallic 60 oxides which are used as catalysts or driers instead, for instance, iron or molybdenum salts, etc. In order to prevent precipitation or settling out of these driers, I may add an "equilibrator" or protective colloid to the mixture and 65 recommend for instance "cadmium resinate", of which about 2% could be added. The mixture is to be kept heated moderately until the ingredients seem thoroughly absorbed.

#### B.—Preparation and ozonization of the main mixture

Of the crude mineral oil or whatever oil residue is to be treated, about 52 per cent of the total finished product have to be taken and slowly 75

heated until about 100° C. are reached. Then the admixture prepared in the first part "A" of the process is added to the mineral oil. Connected by a valve and conduit with the container in which the crude oil is heated and combined with the vegetable oil ingredient, is an ozone generator which can be of any ordinary commercial make, electrically operated or otherwise. After the heating of the oil compound has been maintained around 100° C. for about one hour, a current of nascent ozone is blown through it for approximately another hour.

*C.—Intensified oxidation of alcohol and nitric acid-ageing*

The last phase of the process comprises the addition of an alcohol, such as wood or grain alcohol, diluted in nitric acid, to the mixture, and the quantity added should amount to about 16% of methyl or ethyl alcohol with about 8% concentrated nitric acid in proportion to the total amount of finished product, as predetermined. Likewise, I add a volatile drier, such as spirits of turpentine in the dosage of about 5% of the total. The addition of turpentine, when introduced into the mineral oil previously treated by my process, produces an auto-ebullition lasting about thirty minutes with an escape of gas in the form of a foam amounting in a volume to about 40 percent of the total compound. Such gas when in contact with the atmosphere absorbs strongly oxygen which then is of course embodied into the compound by agitation. The mixture cools off spontaneously after about one hour. This well equilibrated compound is to be left standing for several days without stirring, after which period the finished product can be decanted and filtered through cotton gauze or a similar filtering material. If the ageing period is prolonged, the drying qualities are still improved. Then the product is ready for use or shipment. It may be used entirely in place of linseed oil. The ingredients which in the course of the process enter into the mixture total up as follows:

|                                 | Per cent |
|---------------------------------|----------|
| Crude oil (natural or residual) | 52       |
| Vegetable oil (fatty acids)     | 10       |
| Cadmium resinate                | 2        |
| 50 Lead resinate                | 5        |
| Cobalt resinate                 | 1        |
| Manganese resinate              | 1        |
| Alcohol (methyl or ethyl)       | 16       |
| Nitric acid                     | 8        |
| 55 Turpentine (volatile drier)  | 5        |
| <br>Total                       | <br>100  |

The treatment with nitric acid or the dilution of the alcohol may be modified within a certain range. By numerous experiments I found that I could effect full oxidation of the mineral oil when using nitric acid of 68% of concentration and in a dosage of from 5 to 10%, diluted in alcohol provided in the dosage of 15 to 30%. I furthermore discovered that instead of nitric acid I could use nitrates in their original form or as a derivative, dissolved in alcohol or a similar suitable solvent, either used alone or in combination, to good advantage as far as the promotion of oxidation is concerned, and I therefore claim the right to use nitrates and their derivatives instead of nitric acid, whether they are adapted to develop the acid during treatment or not, for diluting the alcohol used and for the purposes indicated.

It behoves now to consider some of the reactions and transformations taking place in the mixture, while under treatment, more in detail.

While the fatty acids of the liquid glycerines are unsaturated hydrocarbons, the hydrocarbons of the paraffin series or those in the asphaltic mineral oil are saturated and are therefore more or less indifferent to the action of oxygen. However, they are rendered receptive to it by the phenomenon of hydrogenation, which takes place when fatty acids are introduced. These fatty acids, whether isolated or in combination with other unsaturated fats, attack the double or triple atomic carbon structure in the saturated hydrocarbons, and unite with the hydrogen atom, and while becoming thus hydrogenated convert the hydrocarbons thus attached into unsaturated acids. Linolic and linolenic acids, for example, act this way and by taking up oxygen are themselves transformed into resinous substances. Oleic acid deprives the mineral oil of part of its hydrogen and is transformed thereby into solid stearic acid. Even the saturated hydrocarbons of the aliphatic series can be changed into oxidizable products by this hydrogenation.

A further characteristic of the fatty acids is that when they come into contact with pure nitric acid or even with nitrates, they form at various temperatures crystallized stereo-isomers; for example, oleic acid is changed thereby into elaidic acid or elaidin, the elaidic ester of glycerine. These fatty acids therefore have the property to undergo oxidation upon coming into contact with concentrated or diluted nitric acid.

Ozone as an oxidizing agent is much more energetic than simple oxygen, although it should be noted that only the third atom of each ozone molecule plays the active part, while the rest is transformed into plain oxygen.

The strong catalytic power of cobalt is fully realized at the aforementioned temperature of 100° C. and the unsaturated fatty acids of the liquid glycerines are changed into the saturated acids of solid glycerines, ultimately then the oleic, linoleic and iso-linolenic acids are completely transformed into solid stearic acid.

This mineral oil, made oxidizable by the process described can be used entirely like linseed or a similar vegetable oil and can be used as the carrier or base for innumerable anhydrous pigments; for example, zinc oxide, zinc sulphide, lead sulphate or leaded zinc, barium sulphate, white lead, etc., also, if it is derived from more viscous mineral oils, as the base for printing and lithographic inks, stamping inks, etc.

Of the peculiar advantages of this oxidizable mineral oil, whether used alone as a varnish or as a pigment carrier, it may be mentioned that paints prepared with this vehicle dry and oxidize perfectly in from six to eight hours, according to climatic conditions. These paints are likewise weather-resistive, whether exposed to high or low temperatures. Under exposure to solar rays or rain they do not discolor or blacken. Their durability is by no means inferior, if not superior to ordinary vegetable oil paints. The film they form remains durable, solid and flexible, so that it does not crack or plaster off. It is thus obvious that all the listed objects of my invention are fulfilled in a satisfactory, economical and inexpensive way and a perfect cheap substitute for the expensive linseed and similar vegetable oils can be manufactured from almost worthless residues of mineral oils and asphalts.

In accordance with the provisions of the patent statutes, I have described my invention, but I desire it understood that the process is not confined to the particular steps or their sequence, exactly as described, the same being merely illustrative, and that the invention may be carried out in a modified manner without departing from the spirit or leading principles of my inventive concept, and I also claim broadly the right to employ all chemical equivalents, or instrumentalities coming within the scope of the appended claims, and by means of which the enumerated objects of my invention are attained and novel results accomplished, as it is obvious that the particular means herein described, chemicals or quantities listed are only some of many that can be employed according to the same principles and to obtain the same objects and results.

Having now described my invention, what I claim and desire to secure by Letters Patent is:

1. A process of converting a mineral oil into an oxidizable oil, characterized by the following steps: heating said mineral oil to a temperature not substantially above 100° C., incorporating in it approximately up to one-fifth of its quantity of a vegetable oil, containing fatty oxidizable

acids, blowing a current of ozone through the compound for about one hour, while maintaining a temperature of about 100° C., and adding a mixture of nitric acid, diluted in twice its weight of alcohol to the ozonized compound, said diluted acid mixture to be between one third to one-half of the mineral and vegetable oil quantity combined. 5

2. A process of converting a mineral oil into an oxidizable oil, characterized by the following 10 steps: heating said mineral oil to a temperature not substantially above 100° C., incorporating in it approximately up to one-fifth of its quantity of a vegetable oil, containing fatty oxidizable acids, together with a suitable dosage of an 15 oxygenating catalyst, previously admixed, such as lead resinate, cobalt resinate and/or manganese resinate, blowing a current of ozone through the compound for about one hour, while maintaining a temperature of about 100° C., and adding a mixture of nitric acid, diluted in twice its 20 weight of alcohol to the ozonized compound, said diluted acid mixture to be between one third to one half of the mineral and vegetable oil quantity combined. 25

GIOVANNI FIORE.